

## UNITED STATES PATENT OFFICE

JOSEPH M. F. LEAPER, OF BUFFALO, NEW YORK, ASSIGNOR TO THE BARRETT COMPANY, OF NEW YORK, N. Y., A CORPORATION OF NEW JERSEY

## PROCESS OF CONCENTRATING ORES BY FLOTATION

No Drawing.

Application filed January 16, 1928. Serial No. 247,270.

- This invention relates to the separation of minerals and the concentration of ores by flotation processes, and is particularly directed to such separation and concentration, whereby improved results are obtained, by carrying out the flotation operation with the addition to the mineral pulp or ore of a thioformaldehyde, more particularly a polymerized form of thioformaldehyde.
- 10 The thioformaldehyde, or polymerized form of thioformaldehyde, employed in the present invention can be prepared in any suitable or well-known manner, for example, by treating an aqueous or alcoholic solution 15 of hexamethylenetetramine, saturated with ammonia, with hydrogen sulfide (Berichte, vol. 19, p. 2345 (1886)), by treating trimethylenetrisulfoxide with hydriodic acid (J. f. prakt. Chemie, (2), vol. 88, pp. 50-51 20 (1913)), by treating formalin with concentrated alkali metal sulfide to produce trithioformaldehyde (Centralblatt, 1913, II, p. 916), and by treating aqueous solution 25 of sodium thiosulfate with formaldehyde and subsequently adding hydrochloric acid (Berichte, vol. 47, pp. 2562-3 (1914)). The present invention particularly contemplates using the thioformaldehyde, which is called thioform and prepared according to this last 30 method, as a flotation agent. Other methods are also known for making thioformaldehyde and its polymers.
- In carrying out the flotation process, the flotation agent comprising the thioformaldehyde may be incorporated with the ore or the mineral pulp in any suitable manner and at 35 any suitable time which will insure a satisfactory flotation operation. For example, it may be introduced in the free state or it may 40 be dissolved, suspended or dispersed in any suitable solvent or dispersing agent such as, for example, water, or one or more of the usual flotation oils or oil mixtures, or in any suitable organic solvent or medium, and in 45 incorporating the resulting solution, suspension or dispersion with the ore or ore pulp. While a thioformaldehyde shows marked action as a flotation agent, it ordinarily possesses insufficient frothing qualities and 50 is therefore generally used to advantage in conjunction with a suitable or well-known frothing agent, e. g., pine oil, terpineol, tar acids, etc. It may also sometimes be used to advantage in conjunction with other flotation agents.
- The process of the present invention can be carried out in any suitable apparatus, for example, those of the pneumatic type such as the Callowcell, or those where the air is incorporated with the mixture by mechanical agitation such as the Janney apparatus, or the like.
- It is of advantage in many cases, as with certain copper ores, to subject the pulp to the action of an amount of alkali sufficient to give it a neutral or an alkaline reaction before subjecting it to flotation with the aid of a thioformaldehyde. The alkali may be caustic alkali such as caustic soda, or an alkaline salt such as soda ash, or it may be calcium oxide or hydrate, etc.
- The amount of thioformaldehyde required to be used in the flotation process will vary, it depending partly on the character and composition of the ore, partly on the particular thioformaldehyde employed, and partly on other factors. In many cases, one-sixth to one-half of a pound of the thioformaldehyde per ton of ore will be sufficient, while in other cases larger or smaller amounts than this may be required.
- The invention will be further illustrated by the following specific example, but it will be understood that the invention is not limited thereto. The parts are by weight.
- Example: 500 parts of a copper sulfide ore (of the Anaconda Copper Company) assay-ing 1.51 percent copper was ground to a pulp in a ball mill with 215 parts water, 0.75 parts lime, and 0.0625 parts of thioform (prepared according to Berichte, vol. 47, pages 2562-3 (1914)). The ground pulp was diluted with water to give a mixture containing about 16 percent solids and subjected to flotation in a Janney flotation apparatus. After agitating for two or three minutes, a small amount (e. g., about 0.02 parts) of pine oil was added. A satisfactory froth was obtained. During the next 20 minutes of agitation, an amount of pine oil was added sufficient to make a total

of about 0.04 to 0.06 parts. 41 parts of a concentrate assaying 18.61 percent copper was obtained which is a recovery of 88 percent copper. The tailing assayed 0.20 percent copper.

It will thus be noted that the present invention contemplates the utilization of a thioformaldehyde as a flotation agent in the separation of minerals and the concentration of ores; that it may be incorporated with the ore or mineral pulp in any well-known or suitable manner; and that it may be employed in the free state or in solution, suspension or dispersion in any suitable solvent or medium.

It will be understood that the present invention is applicable to the treatment of various kinds of mineral mixtures, both natural and artificial, which are amenable to concentration by flotation processes.

I claim:

1. In the process effecting the concentration of minerals by flotation, the improvement which comprises adding a thioformaldehyde to the mineral pulp and subjecting the resulting mixture to a froth flotation operation.
2. A method of effecting the concentration of minerals by flotation which comprises incorporating thioform with the mineral pulp and subjecting the mixture to a froth flotation operation.
3. In effecting the concentration of minerals by flotation, the process which comprises subjecting a sulfide ore in the form of a pulp to a froth flotation operation in the presence of from about one-sixth to about one-half pound of a thioformaldehyde per ton of ore treated.
4. In effecting the concentration of minerals by flotation, the process which comprises subjecting a copper sulfide ore in the form of a pulp to a froth flotation operation in the presence of from about one-sixth to about one-half pound of thioform per ton of ore treated.
5. In effecting the concentration of minerals by flotation, the process which comprises subjecting a copper sulfide ore in the form of a pulp to a froth flotation operation in the presence about one-fourth pound of a thioformaldehyde prepared by treating sodium thiosulfate in the presence of formaldehyde with hydrochloric acid per ton of ore treated.

In testimony whereof I affix my signature.

JOSEPH M. F. LEAPER.